

Dec. 20, 1927.

1,653,395

J. F. DRISCOLL

PAVEMENT

Filed Feb. 23, 1922



Inventor  
James F. Driscoll  
by George Popp  
Attorneys.

## UNITED STATES PATENT OFFICE.

JAMES F. DRISCOLL, OF BUFFALO, NEW YORK.

## PAVEMENT.

Application filed February 23, 1922. Serial No. 538,681.

This invention relates to a pavement of the kind containing bitumen and commonly known as asphalt pavement, and has for its object the construction of a pavement of this character which has better wearing qualities and can be constructed more economically owing to the reduced cost of equipment, the necessity for less skilled labor and the reasonable price of the materials, which are required.

Heretofore pavements of this type have usually been constructed of soft bitumen or materials having a high bitumen content which was regarded as more durable than one made of harder bitumen or materials having a low bitumen content. While this kind of pavement served fairly well in the past, it no longer is satisfactory for pavements since the advent of the automobile and the motor truck, inasmuch as such vehicles, owing to their high speed and the heavy loads carried by the same, have the tendency to "shove" or produce a "wave" effect on the same, which not only renders the road-way rough and unpleasant but soon destroys the same.

My invention contemplates the use of bitumen which is not so soft as would produce a shoving or waving effect under a moving load, nor so hard that the same would be brittle and readily disintegrate when subjected to a rolling pressure, but instead be of medium viscosity or fluid consistency so that the same will not flow readily and possesses the required stability to hold its shape under varying kinds of traffic and yet be pliable enough to be unaffected by the changes in temperature which effect other composite pavements.

The accompanying drawing is a fragmentary cross section of a pavement constructed in accordance with my invention.

Generally speaking, the roadway embodying my improvement comprises a foundation 1 provided along each of its longitudinal edges with a curb 2, a lower primary coat or body layer 3 arranged over the foundation between the curb, and an upper secondary or course 4 arranged upon the lower layer and forming the sealing coat of the pavement, so as to render the latter water proof.

The lower layer or bottom coat preferably consists of any suitable aggregate ranging in size from impalpable dust to rock passing through a screen of one and a half inch

mesh, the finer material being sufficiently plenty in quantity to produce the least volume of voids between the larger particles such as rock, this being governed by the kinds of materials which are available and used in the pavement.

This layer contains a sufficient quantity of bituminous cement which is mixed with the aggregate commonly known as "metal" so that all particles of the same are thoroughly and completely coated with bitumen and form a homogeneous mass, the mixing of these materials being effected after the same are heated in any well known and approved manner.

The first or bottom course after being deposited on the foundation is spread by raking or otherwise while hot and pliable enough to be manipulated so that the same is of the proper thickness over the entire foundation. This bottom coat or lower layer after being thus spread uniformly is now pressed down very lightly either by rolling or tamping and just sufficient to turn down the pointed sections or jagged ends of the particles of rock or other coarse material in the lower layer without however appreciably compressing the bottom layer and thus leave the upper surface of the same more or less rough and in the best condition to receive the upper layer or second coat of the pavement.

After the lower layer has been thus rolled or tamped lightly and while the same is still hot the upper layer or superficial course which operates as a seal coat is spread over the lower layer to a uniform depth of about one-half to one inch. The spreading of the seal coat is effected while the same is hot and pliable enough to be easily manipulated. This seal coat consists of a finer material or aggregate than the first coat or bottom course and may range from impalpable dust or Portland cement to a sand or screenings which would pass through a sieve having a one-half inch mesh so as to form a mixture with the least volume of voids. This aggregate is mixed with a bituminous cement of the same consistency as that in the lower layer, being neither softer nor harder and this mixing is effected after the bitumen and aggregate having been properly heated, so as to form a homogeneous mass.

While both layers or courses of the pavement are still hot enough to be easily manipulated or worked the same are subjected

to a downward pressure by means of a roller, tamper or other suitable device, this pressure being greater than the initial pressure previously applied to the lower layer 5 alone and sufficiently heavy to compress both layers so effectively that the two layers will be practically amalgamated or merged into each other with no joint or division between them while at the same time both 10 layers are condensed or compacted throughout the entire mass or thickness of the same, and thus form practically a single layer which is sufficiently rigid to resist wear and tear as well as displacement.

15 It will be readily seen that in applying a pressure by a roller or tamper which is sufficiently light to merely turn over or flatten the projecting points or edges of the loose particles of rock appearing on or near 20 the surface of the bottom course after it has been spread or raked and while it is still hot it is possible to lay a sealing course over the same which is practically uniform in thickness, and into which no great amount of 25 rock is projecting upwardly which otherwise would leave the upper sealing course thick in some places and of practically no thickness whatever in others so far as the upper layer is concerned. By thus avoiding 30 sharp upward projections into the seal coat of the wearing course of the pavement this seal coat is not liable to become indented by the traffic running over the same, nor start to wear unduly rapid at these points of indentation which would permit dislodgement 35 of the rock or metal, but instead provides a

uniform covering over which the weight and wear of the traffic is distributed evenly and rapid deterioration is avoided.

By employing bitumen of the same consistency in both layers or courses, the changes in temperature have the same effect on both layers, thereby avoiding any tendency of the two layers to separate as would be the case if the bitumen in these 45 layers were of different consistency.

I claim as my invention:

The herein-described method of making a pavement which consists in laying on the foundation a lower body layer consisting of 50 a mixture of bitumen, a fine mineral aggregate and a coarse mineral aggregate while this mixture is hot; light rolling this body layer while hot so as to moderately compact the same and turn over the points of any of 55 the course aggregate which may project upwardly after being laid on the foundation and thereby cause the coarse aggregate to face upwardly with its wide surfaces; applying an upper finishing layer consisting 60 of bitumen and fine mineral aggregate while hot over said lower layer while the latter is still hot; and then subjecting the upper and lower layers while still hot to a heavy 65 rolling so as to compact the same and weld these layers together into one integral mass in which no line of division is present between the lower and upper layers and the upper and lower surfaces of the pavement are sealed against the entrance of water.

JAMES F. DRISCOLL.